

## UNITED STATES PATENT OFFICE

LEROY C. STEWART AND LEE DE PREE, OF MIDLAND, MICHIGAN, ASSIGNORS TO THE DOW CHEMICAL COMPANY, OF MIDLAND, MICHIGAN, A CORPORATION OF MICHIGAN

## METHOD OF STABILIZING CHLORINATED ALIPHATIC HYDROCARBONS

No Drawing. Application filed June 22, 1932. Serial No. 618,693.

The invention relates to methods of inhibiting the decomposition of chlorinated aliphatic hydrocarbons and to the improved product thereby obtained.

5 The marked tendency of chlorinated aliphatic hydrocarbons, e. g. carbon tetrachloride, tetrachloroethylene, propylene chloride, etc. toward decomposition during storage and/or distillation, particularly in the presence of moisture, is well known. In general this tendency toward decomposition is more pronounced when such hydrocarbons are in contact with copper, as during distillation in dry cleaning solvent recovery, etc. Furthermore, in connection with the distillation of the aforementioned chlorinated hydrocarbons in copper recovery stills, it has been shown that by inter-action between the decomposition products of the hydrocarbons and the 20 metal of the still, copper salts are formed which markedly accelerate the decomposition of the hydrocarbon. Thus the rate at which the solvent breaks down increases progressively when in contact with copper. Such decomposition quite generally imparts to the chlorinated hydrocarbons corrosive properties which render them objectionable for many purposes.

To overcome this difficulty it has been proposed to add to the chlorinated hydrocarbons certain materials which are capable of inhibiting the tendency thereof toward decomposition. For example, chlorinated aliphatic hydrocarbons having incorporated therewith 35 compounds such as benzaldehyde, cyclohexane, various dyes, petroleum oil fractions, toluene, etc. have been proposed as compositions of matter wherein the tendency of chlorinated hydrocarbon toward decomposition is suppressed. However, the use as decomposition inhibitors of compounds such as the foregoing has been disadvantageous, principally because of the relatively large proportion of the inhibitor that must be included with the 40 chlorinated hydrocarbon to render it effective. Other disadvantages, such as coloration of the mixture of inhibitor and hydrocarbon, as in the case of dyes; separation of the inhibitor and hydrocarbon during distillation; as in the 45 case of benzaldehyde, etc.; have attached to

the use of the type of inhibitors, hereinbefore recited.

We have now found that chlorinated aliphatic hydrocarbons can be rendered stable during storage and distillation, particularly 55 in copper apparatus, by incorporating therewith a relatively small amount of a mercaptan. Further, we have found that the composition so produced can be distilled without substantial separation of the inhibitor therefrom.

To the accomplishment of the foregoing and related ends, the invention, then, consists of the features hereinafter fully described and particularly pointed out in the claims, the 65 following description setting forth in detail several approved combinations of ingredients embodying our invention, such disclosed means constituting, however, but several of various forms in which the principle of the 70 invention may be used.

The proportions of the mercaptan, which we have found sufficient in admixture with chlorinated aliphatic hydrocarbons to suppress decomposition, is exceedingly small, 75 e. g. between about 0.001 and 0.1 per cent by volume. The selection of the mercaptan in any particular instance will be determined somewhat by the boiling point of the hydrocarbon, since it is desirable that the boiling 80 point of the mercaptan and that of the hydrocarbon be reasonably close together in order that the mercaptan will be retained therein during distillation.

The following Table I shows the results 85 which have been obtained in practicing our invention, using various mercaptans for inhibiting the decompositions of carbon tetrachloride. As a measure of the decomposition occurring in the chlorinated hydrocarbon 90 during contact with copper and iron, we have determined the milligrams of metal corroded away per square decimeter of area exposed to the action of the hydrocarbon at refluxing temperature for 46 hours in the presence of 95 water. The tests were conducted by partially immersing a weighed and measured strip of metal in a measured volume of the chlorinated hydrocarbon containing the inhibitor in a round-bottomed flask, adding 100

about 40 per cent by volume of water to the mixture in the flask, connecting the flask to a refluxing column; and heating the contents of the flask at refluxing temperature. The amount of inhibitor employed is shown in per cent by volume of the carbon tetrachloride.

Table I

| 10 | Inhibitor          | Percent used | Milligrams loss per square decimeter |       |
|----|--------------------|--------------|--------------------------------------|-------|
|    |                    |              | Copper                               | Iron  |
| 15 | None               | 0.005        | 14,800                               | 1,900 |
|    | n-butyl mercaptan  | 0.005        | 22                                   | 147   |
|    | Phenyl mercaptan   | 0.01         | 27                                   | 296   |
|    | p-cresyl mercaptan | 0.005        | 19                                   | 1,300 |
|    | Ethyl mercaptan    | 0.1          | 19                                   | 267   |
|    | n-heptyl mercaptan | 0.1          | 7                                    | 1,350 |

The decomposition-inhibiting effect of incorporating approximately 0.005 per cent by volume of n-butyl mercaptan with various chlorinated aliphatic hydrocarbons and mixtures thereof is shown in the following Table II, which also gives as the measure of the decomposition occurring in the particular hydrocarbon or mixture the milligrams of copper corroded away per square decimeter of area exposed to the action of the hydrocarbon at refluxing temperature for 46 hours in the presence of water.

Table II

| 35 | Hydrocarbon              | Milligrams loss per square decimeter |           |
|----|--------------------------|--------------------------------------|-----------|
|    |                          | Copper                               | Mercaptan |
| 40 | Carbon tetrachloride     | 14,800                               | 22        |
|    | Tetrachloroethylene      | 412                                  | 7         |
|    | Chloroform               | 231                                  | 70        |
|    | Trichloroethylene        | 92                                   | 25        |
|    | Propylene chloride       | 43                                   | 11        |
| 45 | Mixtures                 |                                      |           |
|    | 50% Carbon tetrachloride | 13,000                               | 236       |
|    | 50% Tetrachloroethylene  |                                      |           |
|    | 50% Carbon tetrachloride | 12,700                               | 25        |
|    | 50% Trichloroethylene    |                                      |           |
|    | 90% Carbon tetrachloride | 10,100                               | 23        |
|    | 10% Propylene chloride   |                                      |           |
| 50 | 90% Tetrachloroethylene  | 830                                  | 17        |
|    | 10% Propylene chloride   |                                      |           |

From the foregoing tables it is readily to be seen that the incorporation of a relatively small amount of a mercaptan with chlorinated aliphatic hydrocarbons results in a distinct reduction of the decomposition occurring in the hydrocarbon when in contact with copper or iron even under the extremely severe conditions of continuous refluxing over a 46 hour period of time in the presence of water. Further, we have determined that a similar benefit inures to the aforementioned hydrocarbons from the admixture therewith of a mercaptan when in contact with other metals, e. g. iron, steel, tin, Monel metal,

zinc, etc. The decomposition resulting in such hydrocarbons upon exposure to sunlight is also generally inhibited in our new composition.

Particularly to be noted is the effect upon the decomposition rate caused by incorporating a mercaptan with carbon tetrachloride, or mixtures thereof with various other chlorinated aliphatic hydrocarbons. The tables show that the addition of only 0.005 per cent of n-butyl mercaptan reduces the amount of corrosion, or, suppresses the decomposition, of carbon tetrachloride to a negligible quantity. Likewise, in mixtures of carbon tetrachloride with various other chlorinated hydrocarbons such as propylene chloride, which in particular seems to accelerate decomposition of the tetrachloride, decomposition is substantially inhibited, and such mixtures may safely be stored or shipped in iron or steel containers.

Among the especially advantageous applications which can be made of our improved composition of matter are (1) dry cleaning, wherein recovery of the solvent composition is accomplished by distillation; and, (2) vapor phase degreasing of metallic articles.

Other modes of applying the principle of our invention may be employed instead of the one explained, change being made as regards the materials employed, provided the ingredients stated by any of the following claims or the equivalent of such stated ingredients be employed.

We therefore particularly point out and distinctly claim as our invention:

1. A composition of matter comprising a chlorinated aliphatic hydrocarbon and a relatively small amount of a mercaptan.
2. A composition of matter comprising a chlorinated aliphatic hydrocarbon and between about 0.001 and 0.1 per cent by volume of a mercaptan.
3. A composition of matter comprising a chlorinated aliphatic hydrocarbon and about 0.005 per cent by volume of n-butyl mercaptan.
4. A composition of matter comprising carbon tetrachloride and a relatively small amount of a mercaptan.
5. A composition of matter comprising carbon tetrachloride and about 0.005 per cent by volume of n-butyl mercaptan.
6. A composition of matter comprising tetrachloroethylene and a relatively small amount of a mercaptan.
7. A composition of matter comprising tetrachloroethylene and about 0.005 per cent by volume of n-butyl mercaptan.
8. A composition of matter comprising trichloroethylene and a relatively small amount of a mercaptan.
9. A composition of matter comprising trichloroethylene and about 0.005 per cent by volume of n-butyl mercaptan.

10. The method of inhibiting the decomposition of chlorinated aliphatic hydrocarbons which consists in incorporating therewith a relatively small amount of a mercaptan.

11. The method of inhibiting the decomposition of chlorinated aliphatic hydrocarbons which consists in incorporating therewith between about 0.001 and 0.1 per cent of a mercaptan.

12. The method of inhibiting the decomposition of chlorinated aliphatic hydrocarbons which consists in incorporating therewith about 0.005 per cent of n-butyl mercaptan.

13. A composition of matter comprising a chlorinated aliphatic hydrocarbon which has at least two chlorine atoms in the molecule and a relatively small amount of a mercaptan.

14. The method of inhibiting the decomposition of chlorinated aliphatic hydrocarbons having at least two chlorine atoms in the molecule which consists in incorporating therewith a relatively small amount of a mercaptan.

Signed by us this 17th day of June, 1932. 75

LEROY C. STEWART.  
LEE DE PREE.

80

20

85

25

90

30

95

35

100

40

105

45

110

50

115

55

120

60

125

65

130